

Patented Feb. 14, 1928.

1,659,396

# UNITED STATES PATENT OFFICE.

WILLIAM A. DOUGLASS, OF PENNS GROVE, NEW JERSEY, ASSIGNOR TO E. I. DU PONT DE NEMOURS & COMPANY, OF WILMINGTON, DELAWARE, A CORPORATION OF DELAWARE.

## PROCESS OF CONCENTRATING ORES AND MINERALS BY FLOTATION.

No Drawing.

Application filed October 25, 1926. Serial No. 144,193.

This invention relates to the recovery of valuable ores and minerals by flotation, and comprises more particularly the concentration of such ores and minerals by means of a certain class of organic flotation agents.

It is one of the objects of the present invention to carry out flotation processes in an efficient manner by using as the flotation agent one of a class of organic compounds having highly selective properties when so used. It is a further object to carry out the flotation processes by using flotation agents which are suitable for use in neutral, alkaline or acid flotation circuits without dependence of the flotation agents.

I have discovered that these and other objects may be accomplished by using in a flotation process organic derivatives of trithio carbonic acid as the flotation agents. These compounds are characterized by having the following general structural formula:



where R and R' are organic groups. R and R' may represent the same or different organic groups.

A specific example of a derivative in which R and R' are alkyl groups is diethyl ester of trithio carbonic acid having the following formula:



An example of a derivative in which R and R' are substituted alkyl groups is B-B trithio carbonyl ethyl acetate having the following formula:



Dibenzoyl trithio carbonate having the formula:



is an example of a derivative in which R and R' are acyl groups. Diethyl thiol ester

of thion carbonyl disulfide having the following formula:



55

is still another type of derivative of trithio carbonate, wherein R is an alkyl group and R' is another trithio carbonate group having the following formula:



65

in which X represents an organic group such as an alkyl.

The various derivatives of trithio carbonic acid may be made in any suitable manner. For instance, diethyl trithio carbonate can be made by dissolving 150 grams of potassium hydroxide in 250 cc. water, and saturating this solution with hydrogen sulfide. To this solution is added 150 grams of potassium hydroxide and when all is dissolved, 250 grams of carbon bisulfide are added and the mixture agitated vigorously until all of the carbon disulfide goes into solution. The solution is washed once with 300 cc. of alcohol. To the water layer containing potassium trithio carbonate, 300 grams of ethyl bromide are slowly added with agitation and cooling. The reaction product is washed with water and the excess ethyl bromide removed by bubbling a current of air through the liquid. The resulting orange red liquid is pure diethyl trithio carbonate.

This compound may be used as a flotation reagent in the following manner: 500 grams of minus 29 mesh Phelps-Dodge Corporation Copper Queen ore are ground for 20 minutes in a pebble mill with 500 cc. of water, 0.6 grams of lime and 0.025 grams of diethyl trithio carbonate. The lime and diethyl trithio carbonate are in the proportions of 2.4 lbs. and 0.10 lb. respectively per ton of ore. The pulp from the pebble mill is transferred to a Janney laboratory flotation machine and a frothing agent (terpineol or pine oil) added. The pulp is diluted to about two liters and a rougher concentrate removed.

75

80

85

90

95

100

for 10 minutes, water being added as needed. The following results were obtained:

% Cu in concentrate=7.25.  
% Cu in tailings=.22.  
Extraction=87.6%.

Using Anaconda Table Tailings in a neutral circuit with diethyl trithio carbonate as the flotation reagent in the proportion of 0.15 lbs. per ton of ore, the following results

10 were obtained:

% Cu in heads=1.88.  
% Cu in concentrate=8.84.  
% Cu in tailings=0.18.  
Total Cu recovered=92.3%.

15 The flotation reagents forming part of the present invention do not decompose in an acid solution, and are therefore suitable for use in acid flotation circuits. Using as the flotation reagent diethyl trithio carbonate 20 in the proportion of 0.15 lbs. per ton of ore in a circuit containing 7.0 lbs. of sulfuric acid per ton of ore, the following results were obtained:

% Cu in heads=1.88.  
25 % Cu in concentrate=9.68.  
% Cu in tailings=0.085.  
Total Cu recovered=96.3%.

30 Dibenzoyl trithio carbonate can be made conveniently by treating potassium trithio carbonate in benzene suspension with benzoyl chloride, removing the heat of reaction by cooling. After filtration from the potassium chloride and evaporation of the solvent, dibenzoyl trithio carbonate is obtained as a 35 yellowish orange oil.

When tested as a flotation reagent using an alkaline circuit according to the process described, the following results were obtained:

40 % Cu in concentrate=6.67.  
% Cu in tailings=.20.  
Extraction=89.2%.

45 Diethyl thiol ester of thioncarbonyl disulfide may be made by treating the mono ethyl ester of trithio carbonic acid (Chancel Jahres bericht für Chemie 1851, p. 513) with iodine. The orange brown oil which is formed, is washed with water and then dried with calcium chloride.

50 When tested as a flotation reagent using an alkaline circuit according to the process described, the following results were obtained:

% Cu in concentrate=6.60.  
55 % Cu in tailings=0.24.  
Extraction=86.9%.

56 In illustrating the present process, reference has been made specifically to certain ores and reagents, and to various specific 60 conditions of operation. It will be understood that the present process is not limited to the specific substances or details of

procedure mentioned, but includes generally processes of recovering values from ores by flotation in which the flotation agents are 65 members of the class of compounds described. For instance, it has been pointed out as being desirable to add a frothing agent in the specific examples noted. However, where the flotation agent itself has 70 sufficient frothing power, the frothing agent may be omitted.

Any suitable modifications and changes may be made without departing from the spirit and scope of the invention.

I claim:

1. In the process of concentrating ores and minerals by flotation the step which comprises subjecting the ore in the form of a pulp to a froth flotation operation in the 80 presence of an organic derivative of trithio carbonate.

2. In the process of concentrating ores and minerals by flotation, the step which comprises subjecting the ore in the form of a 85 pulp to a froth flotation operation in the presence of an organic derivative of trithio carbonate having the following structural formula:



90

where R and R' are organic groups.

3. In the process of concentrating ores and minerals by flotation, the step which 95 comprises subjecting the ore in the form of a pulp to a froth flotation operation in the presence of an organic derivative of trithio carbonate having the following structural formula:



100

where R and R' are the same organic group.

4. In the process of concentrating ores and minerals by flotation, the step which 105 comprises subjecting the ore in the form of a pulp to a froth flotation operation in the presence of an organic derivative of trithio carbonate having the following structural formula:



110

in which R is an alkyl group and R' is an organic radical.

5. In the process of concentrating ores and minerals by flotation, the step which comprises subjecting the ore in the form of a 120 pulp to a froth flotation operation in the presence of diethyl trithio carbonate.

In testimony whereof I affix my signature.

WILLIAM A. DOUGLASS.